# EUROPEAN PATENT SPECIFICATION

(11) **EP 0 121 343 B1**
(45) Date of publication and mention of the grant of the patent: **18.05.1988**
(21) Application number: 84301391.3
(22) Date of filing: 02.03.1984
(51) Int. Cl.: C10G 1/04

(54) **Integrated ionic liquefaction process**
Integriertes ionisches Verflüssigungsverfahren
Procédé de liquéfaction ionique intégré

(30) Priority: 03.03.1983 US 471731; 27.12.1983 US 564223
(43) Date of publication of application: 10.10.1984
(73) Proprietor: PENTANYL TECHNOLOGIES, INC., Boulder Colorado 80303 (US)
(72) Inventor: Bain, Richard L., Lakewood Colorado 80228 (US); Rastle, Charles M., Boulder Colorado 80302 (US); Porter, Clifford R., Arvada Colorado 80004 (US); Kaesz, Herbert D., Los Angeles California 90049 (US)
(74) Representative: Sommerville, John Henry

(56) References cited:
- GB-A- 2 075 046
- GB-A- 2 085 917
- US-A- 4 085 029

## Description

This invention relates to the liquefaction of carbonaceous materials and in particular to a method of producing useful products, including fuel products which can be used directly in petroleum-like refining processes, or as a feed stock for further chemical synthesis, or as a low sulfur fuel oil or the like, and, pseudo-plastic products with melting points in the range of from about 100°C to 200°C which are solid products at ambienttemperature and are characterized by their reduced sulfur and ash content which make them useful as fuel and coke substitutes.

One of the principal approaches to coal liquefaction and solvation in the past has employed reactions producing free radicals through thermal bond rupture. For many kinds of coal used this typically required temperatures above about 350°C for enough free radicals to form through thermal bond rupture of carbon- carbon bonds, carbon-oxygen bonds, carbon-nitrogen bonds and carbon-sulfur bonds, to react with other compounds or hydrogen in order to form lower molecular weight compounds than the complex materials present in the coal. In some typical prior processes the free radicals formed were stabilized and hydrogenated by hydrogen atoms through hydrogen transfer from solvent donor molecules such as 1,2,3,4-tetrahydronaphthalene or 9,10-dihydrophenanthrene, often used in the presence of minor amounts of coal solubilizing agents. After such reactions the solids are generally separated by distillation, or by solvent deashing. For such systems to be effective, it is important that the mixtures be suitable for either effective distillation or deashing without excessive coking. In processes where even minor amounts of highly polar solvents are employed either in the liquefaction reactor or subsequently, distillation problems are encountered and when alkali compounds are present, severe coking problems can arise.

In one embodiment, the present invention uses a mixture of carbonaceous material, polar solvent, and alkaline compounds to produce liquid and solid products by a process which will be referred to herein as ionic liquefaction. The resulting products, both liquids and solids are then separated in various process embodiments from the unreacted carbonaceous material. The products are separated and stabilized in a manner which minimizes the deleterious effects normally encountered in the distillation, separation, and stabilization of mixtures containing polar organic liquids and alkaline compounds. It is therefore an object of this invention to produce and separate liquid and solid products from carbonaceous materials, in liquefaction processes which employ mechanisms other than the formation of free-radicals. This invention provides a method for liquefaction that is characterized by reaction conditions which do not favor thermal rupture free radical mechanisms and uses primarily ionic chemical mechanisms at lower temperatures and pressures than previously employed to produce useful, novel liquid and solid products. The invention as described contemplates an integrated process for the liquefaction of carbonaceous material starting from the preparation of the feed material to the separation of products, including the recovery and use of recycle streams rich in phenolics. It is a further object of the present invention to produce a novel pseudo-plastic material that is a solid at room temperature, which has reduced sulfur and ash content and which is useful as a fuel, coke or petrochemical feedstock.

These and other objects of the invention together with the features and advantages thereof will become apparent from the following detailed specification when read in conjunction with the accompanying drawings in which like reference numerals refer to corresponding parts, and:
Fig. 1 is a schematic flow chart of a typical integrated ionic liquefaction process useful with the present invention for coal;
Fig. 2 is a schematic representation of a liquefaction subsystem useful with the flow chart of Fig. 1;
Fig. 3 is a schematic representation of a separation subsystem useful with the present invention;
Fig. 4 is a schematic representation of a distillation subsystem useful with the present invention;
Fig. 5 is a schematic representation of a hydrogenation subsystem useful with the present invention;
Fig. 6 is a schematic of an acid hydrolysis subsystem useful with the present invention;
Fig. 7 is a schematic of another acid hydrolysis subsystem useful with the present invention;
Fig. 8 is a schematic flow chart of another typical ionic liquefaction process using acid hydrolysis useful with the present invention;
Fig. 9 is a schematic flow chart of another typical ionic liquefaction process using coking useful with the present invention;
Fig. 10 is a schematic flow chart of another integrated ionic liquefaction process useful for the production of a pseudo plastic solid fuel and coke substitute;
Fig. 11 is a schematic illustration of a liquid-liquid solvent extraction system useful in the process shown in Fig. 10; and
Figs. 12 to 14 are a series of graphic representations showing carbon monoxide conversions and temperature profile plotted against time for a series of experimental runs according to the teachings of the present invention.

As used herein, the term carbonaceous material, includes solid, semi-solid and liquid organic materials which are susceptible to the described treatment methods. Examples of solid carbonaceous materials which may be used in connection with the practice of the present invention include coal, such as anthracite, bituminous, subbituminous and lignite coals, as well as other solid carbonaceous materials, such as wood, lignin, peat, solid petroleum residuals, solid carbonaceous materials derived from coal, and the like, depending on the products sought. Examples of semi-solid and liquid carbonaceous materials include coal tars, tar sand, asphalt, shale oil, heavy petroleum oils, light petroleum oils, petroleum residuals, coal derived liquids and the like.

Ionic liquefaction as used herein is intended to mean the chemical process described herein, which is characterized by polar solvent solubilization of the polymeric structure of carbonaceous materials susceptible to the described treatment methods, in the presence of alkali and alkaline earth compounds in amounts which favor ionic reactions involving the solubilized carbonaceous material and ionic species such as phenoxide, hydroxide, and formate ions, and favor stabilization of the ionic species to produce distillable products, low-sulfur fuel oils, and low-ash reduced-sulfur pseudo-plastic, normally solid products useful as fuel, coke, or petrochemical feedstock.

In addition to ionic reactions, it is believed that ionic liquefaction, as described herein, may change the apparent molecular weight and other physical properties of the solubilized carbonaceous material by reducing the extent of hydrogen bonding between carbonaceous material molecules. Because of the reactive nature of ionic species remaining after solubilization and ionic reaction, the product mixture must be further processed in order to stabilize the desired products to be able to recover liquid and solid usable products including a recycle stream rich in phenolics which can be used in the ionic liquefaction reactor. This processing involves removal of alkaline salts, and further stabilization of organic ionic species by hydrogenation, acid hydrolysis, solvent extraction or coking.

The term alkaline as used generally and herein is synonymous with basic which includes, without limitation, alkali metal and alkaline earth compounds. A base can be an aqueous solution which contains OH- ions, or any substance which accepts protons, or any substance which is an electron pair donor. Typical cations are the light metals of Groups IA and IIA of the Periodic Table. Preferred cations are Na⁺ and K^{+.} Typical anions include OH⁻, C0₃-, HCO_{Z}-, and HC0₃^{-.}

As applied to ionic liquefaction a polar solvent or polar solvents means a solubilizing agent selected from the group consisting of aromatic alcohols, phenols, polycyclic phenols and substituted phenols, and mixtures thereof. Typically, such solvents do not have an a-hydrogen. Liquid mixtures of solubilizing polar solvents used in the ionic liquefaction process of the present invention typically will contain greater than 50% by weight of such polar solvents.

More particularly, in accordance with a preferred embodiment of the invention, useful hydrocarbons are obtained from carbonaceous materials by contacting the carbonaceous materials with a solvent/solute system consisting of (a) an organic phase comprising a solubilizing agent containing more than about fifty percent (50%) by weight of a phenolic-type solvent such as an aromatic phenol, polycyclic phenol, substituted phenol or a mixture thereof, and (b) an inorganic phase comprising an aqueous solution of one or more alkali or alkaline-earth metals. More particularly, the solvent/solute system comprises one or more solubilizing agents selected from aromatic phenolics, e.g. phenols, and polycyclic and/or substituted phenols, typically of from 6 to 15 carbon atoms, e.g. o-cresol, m-cresol, p-cresol, catechol; resorcinol, naphthol, and mixtures and derivatives thereof. Although not essential to the practice of this preferred embodiment of the invention other organic constituents such as aromatic alcohols, polycyclic aromatic hydrocarbons, partially hydrogenated and/or fully hydrogenated polycyclic aromatic hydrocarbons, typically having from 1 to 4 carbon rings, and more preferably from 2 to 3 carbon rings e.g. naphthalene, anthracene, phenanthrene, Tetralin (tetrahydronaphthalene), gamma-picoline, isoquinoline, dihydronaphthalene, Decalin (decahydronaphthalene), 9,10-dihydroanthracene, 9,10-dihydrophenanthrene, and mixtures and derivatives thereof, also may be included in the solvent/solute system.

Synthesis gas, as that term is used herein, means a gas primarily comprised by carbon monoxide and hydrogen. Other gaseous components present in small concentrations can include carbon dioxide, light hydrocarbon gases, and some impurities such as nitrogen and still be effective in the process described herein. In addition, small amounts of water vapor may also be present.

It has been shown that solubilization of coal and other carbonaceous materials can be achieved using a variety of coal derived solvents and other organic solvents. For example, U.S.-A-4,133,646 teaches the advantages of using minor amounts of phenolic recycle solvents in coal liquefaction. Similar advantages are taught by Kamiya et al., "Effect of Phenolic Compounds on Liquefaction of Coal in the Presence of Hydrogen-Donor Solvent", Fuel, Vol. 57 (November 1978), pp 681-685; and by Sams, et al., "Internal Rearrangement of Hydrogen During Heating of Coals with Phenol", Fuel, Vol. 60 (April 1981 pp 335-341. It is also known that the use of various alkali bases, e.g. NaOH, Na2CO3 and NaHC0₃, are useful in carbonaceous liquefaction processes. See for example, Donovan et al., "Oil Yields from Cellulose Liquefaction", Fuel, Vol. 60 (October 1981), pp. 899-902 and Araya et al., "Study of Treatments of Subbituminous Coals by NaOH Solutions", Fuel, Vol. 60, (December 1981), pp 1127-1130.

Ross and Blessing have described how coal may be solubilized and hydrogen added to the organic product by aqueous base "Hydroconversion of a Bituminous Coal with CO-H₂0", Fuel, Vol. 57 (June 1978), p. 379. They have also described how alcohols having an a-hydrogen atom are effective hydrogen donor solvents when catalyzed by alkaline compounds (U.S.-A-4,298,450). They state, however, that alcohols not having an a-hydrogen are not effective solvents.

The unexpectedly high solubilization and liquefaction achieved in the present invention through the synergistic effect in a liquefaction reactor of a solvent/solute system combining a phenolic solvent, water and added amounts of an alkali or alkaline-earth metal compound, with or without the addition of synthesis gas, depending on the reactants selected, has made possible the investigation and discovery of other promising opportunities for enhancing the liquefaction and the hydrogen to carbon ratio of the resultant products, which will be more fully described hereinafter.

Appell et al., in their paper entitled "On the Mechanism of Lignite Liquefaction with Carbon Monoxide and Water", Chem. and Ind., VoI. 47, (1967), p. 1703, describe how using freshly powdered low-rank coal and a selected solvent will produce a 72% yield of a benzene-soluble oil when using operating pressures near 5000 psig and temperatures in excess of 365°C. Appell et al., also describes the use of a solvent comprising alpha-naphthol (a phenol), phenanthrene (a polycyclic aromatic hydrocarbon) and water in the presence of naturally occurring amounts of alkali or alkaline-earth metal compounds at similar operating conditions. In addition testing is described involving the addition of K₂CO₃ in water as a solvent with the conclusion that the addition of K₂C0₃ increases the extent of the water gas shift reaction but is not believed to significantly improve hydrogen uptake by the coal during liquefaction under the conditions employed.

Farcasiu et al, U.S. Patent No. 4,133,646 (1979) teach that an improved liquefaction process can be obtained using a two-stage liquefaction process wherein a donor solvent in combination with minor amounts of phenolic compounds is reacted with coal and hydrogen at 315-454°C (600-850°F)- The unreacted coal was recovered by filtration, phenolic compounds were recovered by distillation, or extraction, and the resulting substantially phenolic free distillation residue was subjected to various upgrading treatments such as delayed coking and hydrotreating.

Farcasiu et al, did not obtain the synergistic effect realized by the present invention using solvents containing greater than 50% by weight of phenolic compounds with added alkaline compounds in a single stage liquefaction reaction. Farcasiu et al, similarly also did not recognize that phenolic compound recovery from the product stream must be preceded by alkaline compound removal. Likewise, Farcasiu et al does not show how alkaline compound separation may be controlled by varying the water level during the added alkaline compound removal step. Further, there is no disclosure in Farcasiu et al of how the process could be advantageously improved by adding synthesis gas to the first stage reaction, either as a reactant in the formate ion chemistry described hereinafter, or to produce a hydrogen enriched stream for upgrading operations. Beside the foregoing, Farcasiu et al does not disclose that residues containing more than about 50% by weight phenolics may be upgraded by hydrotreating or coking, but instead indicates that the residue should be substantially phenol free.

The foregoing and other art, in summary, has not recognized that a liquefaction process for coal or other carbonaceous material can be substantially improved by the use of an organic solvent containing greater than 50% by weight of phenolic compounds in amounts between about 1.5 to 5.0 times the weight of carbonaceous materials, in combination with between 25 to 400 parts by weight of alkali for every 1000 parts by weight of carbonaceous material, and between 25 to 400 parts by weight of water for every 1000 parts by weight of carbonaceous material; when the carbonaceous material, the organic solvent and the solvent/solute pair are reacted together at temperatures less than about 360°C and pressures between about 300 psia (2.06 MPa) to about 2500 psia (17.2 MPa). Further improvement can be obtained by the presence of synthesis gas having a H₂1C0 ratio between about 0.5 and 2.0 in amounts between about 0.16 to about 1.25 m³/Kg of carbonaceous material when combined with stabilization of the reaction product before further upgrading, after removal of the alkali and water.

More particularly, in accordance with a preferred embodiment of the invention the solvent/solute systems useful in the practice of the invention are solubilizing mediums comprising organic and inorganic fractions or constituents which may solubilize a portion of the carbonaceous material and/or may otherwise enhance liquefaction of the carbonaceous material. As noted supra, the organic fractions of the solvent/solute systems comprise one or more solubilizing agents selected from the group consisting of aromatic phenolics, e.g. phenols, and polycyclic and/or substituted phenols, typically of from 6 to 15 carbon atoms, e.g. o-cresol, m-cresol, p-cresol, catechol, resorcinol, naphthol, and mixtures and derivatives thereof. Although not essential to the practice of this embodiment of the invention the solvent/solute systems in many instances will include other organic constituents. Suitable organic constituents include aromatic alcohols, polycyclic aromatic hydrocarbons, partially hydrogenated and/or fully hydrogenated polycyclic aromatic hydrocarbons, typically having from 1 to 4 carbon rings, and more preferably from 2 to 3 carbon rings e.g. naphthalene, anthracene, phenanthrene, acenaphthene, 1-methylnaphthalene, 2-methylnaphthalene, Tetralin (tetrahydronaphthalene), gamma-picoline, isoquinoline, dihydronaphthalene, Decalin (decahydronaphthalene), 9,10-dihydroanthracene, 9,10-dihydrophenanthrene, and mixtures and derivatives thereof.

During initial phases of operation, some of the above mentioned solubilizing agents and/or other organic constituents will be present: then in subsequent operation, the organic constituents will be carbonaceous material-derived phenols of the type, and polycyclic aromatic hydrocarbons of the type, or derivatives related to the type, described hereinbefore. Particularly useful organic phase solubilizing agents and/or other organic fraction constituents have a boiling point above 50°C, more preferably of from 100°C to 460°C, and most preferably of from 150°C to 400°C. In the practice of this latter embodiment, the solubilizing agent is typically from about 50 to 100 weight percent of the organic fraction of the solvent/ solute system. Suitable inorganic fraction constituents of the solvent/solute system include water, and alkali and/or alkaline-earth metal compounds, and their derivatives. The water content can be from 5 parts to 60 parts per 400 parts by weight of the solvent/solute system, more usually 15 parts to 40 parts per 400 parts by weight of the solvent/solute system.

Suitable examples of alkali and alkaline-earth metal compounds include hydroxides, carbonates, bicarbonates, nitrates, sulfates, sulfites, sulfides, formates and other salts, mixtures thereof, and the like, although other compounds may be employed for the purpose. Specific examples include NaOH, Na₂C0₃, NaHC0₃, Na₂S0₄, NaN0₃, KOH, K_{Z}C0₃, KHC0₂, CaC0₃, mixtures thereof and the like. Presently preferred species are NaOH, KOH and Na₂CO₃ in from about 1 part to about 40 parts per 400 parts by weight of the solvent/solute system, more usually 1 to about 15 parts per 400 parts by weight of the solvent/solute system. It is understood that the amount of alkali or alkaline-earth metal compound present for purposes of the present invention is an added amount, i.e. an amount in excess of the amount which would be present from the various naturally occurring alkali or alkaline-earth metal compounds. Further, it is understood that the alkali or alkaline-earth metal compound content will be maintained at the desired level in a recycle solvent stream. As will be seen in Example VI et seq., the combination of organic and inorganic fractions and constituents provide a beneficially synergistic effect on solubilizing of carbonaceous material.

The amount of the solvent/solute system required in the reaction mixture or slurry is dependent upon the amount and nature of the carbonaceous material to be treated. Generally, it is preferred to employ up to about 500 parts of the sotvent/sotute system to 100 parts of carbonaceous material, more preferably at least about 350 parts of solvent/solute to 100 parts of carbonaceous material, and most preferably at least 150 parts of solvent/solute system to 100 parts of carbonaceous material.

According to this embodiment, carbonaceous material is solubilized in the solvent system - alkali medium to form a reaction mixture or slurry. Frequently, the reaction conditions are water gas shift reaction conditions, as hereinbefore described.

The reaction mixture is heated to a sufficient temperature, typically below about 400°C, and pressure to obtain enhanced solubilizing of the carbonaceous material for production and/or conversion of hydrocarbon liquids, as hereinbefore defined, from the carbonaceous material. For most purposes, it is contemplated that sufficient temperature levels for the solvent/solute system are from 100°C to a temperature below 400°C under the reaction conditions employed, more preferably from 140°C to 380°C, and most preferably from 260°C to 360°C, at a pressure of at least 300 psia (2.06 MPa), more preferably from about 500 psia (3.45 MPa) to 2500 psia (17.2 MPa), and most preferably from 500 psia (3.45 MPa) to 1500 psia (10.35 MPa). It has been found that under the foregoing reaction condition, relatively short periods of time result in the production of the desired product. Although sufficient times are dependent upon the nature of the carbonaceous material, the reaction conditions employed, and the like, for the most purposes, it is contemplated that reaction times of at least about 1 minute, more preferably from 10 minutes to 120 minutes, and most preferably from 15 minutes to 60 minutes are sufficient to result in enhanced solubilizing and the production and/or conversion of hydrocarbon liquids.

As will be appreciated by those skilled in the art, the solvent/solute systems containing coal or other carbonaceous material solubilized according to the present invention, may be further treated as described herein.

In ionic liquefaction the reaction mechanisms of the chemistry is substantially different than the previously employed reaction conditions which favored thermal rupture-free radical chemical reactions. At the lower temperatures used for ionic liquefaction, the predominant chemistry can be termed as solvation- ionic chemistry, involving solubilization of the coal polymer by polar phenolic solvents, followed in situ by attack upon the coal structure by ionic species such as phenoxide and formate ions. Without being limited to any specific theory, it is believed that the primary points of attack are at the carbon adjacent to oxygen containing functional groups present in the coal. The esters, ketones, and ethers present, are all sites for nucleophilic substitution. Hydroxide and carboxylic acid containing functional groups are considered to be substantially unreactive to nucleophilic substitution. The phenoxide ion mechanism for an ether group is:

The parallel formate ion mechanism V to VII is This mechanism is believed to be enhanced at the mild conditions employed because of the intimate contact made possible by the phenolic solvent solubilization where there is competition for available ionic species in the presence of the water gas shift reaction VIII to X. The summation of VIII, IX and X is the net water gas shift reaction XI:

Ionic liquefaction, therefore, offers many process advantages over conventional thermal rupture free radical liquefaction. The temperature regime for ionic liquefaction is typically under 360°C. At these temperatures thermal bond rupture is not the primary mechanism because it proceeds slowly. The lower temperature employed has the effect therefore of reducing the amount of methane, ethylene, ethane, and acetylene produced from 20% to less than 1% of the MAF carbonaceous material.

System pressure for ionic liquefaction can be obtained from the vapor pressure of the solvents alone or by the addition of external pressurized gases. Sufficient pressure is preferably maintained to ensure that a majority of the solvents are in the liquid phase. This is typically 3.45-10.35 MPa (500-1500 psia). The ionic liquefaction mechanism described herein to produce a liquid, can, in addition, use synthesis gas which is composed of carbon monoxide and hydrogen instead of requiring expensive pure hydrogen. This synthesis gas is the fuel for the production of pure hydrogen, therefore the production of pure hydrogen is not needed to obtain the desired improvement in hydrogen to carbon ratios possible in the liquid products of ionic liquefaction.

In free radical liquefaction, a typical mechanism is:

### Thermal Rupture

### Hydrogen Donation

### Solvent Regeneration

In order to promote the Solvent Regeneration reaction, (equation XIV) free radical liquefaction is typically performed using high purity hydrogen at pressures between 13.8-17.2 MPa (2000-2500 psia).

The ionic liquefaction described herein, at the conditions employed, will produce polar products having low molecular weights. The free-radical mechanism will produce mainly non-polar materials. The free-radical type mechanism can, in addition, lead to polymerization reactions which produce undesirable high molecular weight materials. These type of reactions are not favored and therefore avoided in the ionic liquefaction described herein.

The presence of highly polar phenolic compounds, alkali compounds, and the ionic forms thereof, along with the oxygenated compounds desired from the carbonaceous material, during the ionic liquefaction process described herein, can, however, lead to potential processing problems downstream from the liquefaction reaction. Some oxygenated compounds, including many phenols, are often thermally unstable, especially in the presence of coking promoters such as ionic alkaline species. These compounds are concentrated in the bottoms during distillation operations. It is, therefore, important to minimize the amount of alkaline compounds present in the distillate feed stream. A major proportion of the alkaline compounds should, therefore, be removed before distillation is begun.

In addition, the proposed phenoxide ion chemistry shows a solvent incorporation step as an inherent part of the reaction mechanism. Under the conditions typically used in ionic liquefaction, i.e., relatively low temperature and low pressure, it is difficult for the solvent regeneration reaction IV to proceed to completion. Therefore, to regenerate solvent and obtain additional product, a portion of the liquefaction product liquids should preferably undergo further reaction in the presence of hydrogen under conditions which will break the ether bond between the phenoxide ion and the coal derived organic species. The reaction may be performed at conditions which are severe enough to break the ether bond, but are not severe enough to saturate the aromatic ring, or remove the oxygen atom as water. The hydrogenation, acid treatment or solvent extraction steps will also serve to stabilize the product by reducing the concentration of the most unstable ionic species and reduce the ash content of the product.

Because the ionic liquefaction products produced by the liquefaction processes described are typically high in reactive oxygenated species there can be a tendency for the products to oxidize and/or polymerize with time or with thermal treatment. In the case where additional solvent recovery and product upgrading are necessary, specific sequential processing steps are then needed. A process incorporating these necessary steps is shown in Figure 1.

Referring to the schematic diagram in Fig. 1, the feed preparation at (A), comminutes the carbonaceous material, stream (1), by conventional means such as hammermills or ball mills or comparable equipment; and adds a water-alkali mixture stream (4); and recycle polar solvent streams (2) and (3), containing greater than 50% by weight of phenolic species. The comminution process may be accomplished either dry or wet. If performed wet, then the recycle polar solvent may be used as the wetting agent, if proper precautions are taken. The carbonaceous feed is preferably comminuted to 100 percent minus 74 micron (200 mesh) particle size, more preferably to 100 percent minus 147 microns (100 mesh) particle size, and most preferably to 100 percent minus 350 microns (40 mesh) particle size but in any event must be in a form which will enable the requisite solubilization for the ionic liquefaction to proceed.

Using 1000 parts by weight of stream (1) carbonaceous material as an example, the preferred amount of polar recycle solvent for the required solubilization to proceed, recycle streams (2) plus (3) is between 1500 and 3500 parts by weight depending on the prepared form of the carbonaceous material, with 2000 parts by weight of solvent the most preferred amount. The polar recycle solvent contains preferably greater than about 50% by weight of phenolic compounds, and more preferably greater than 60% by weight phenolic compounds.

The preferred amount of alkaline material in water-alkali mixture stream (4) is selected to be enough to produce the desired results. It has been found under the conditions disclosed herein that between about 25 parts and 400 parts by weight per 1000 parts by weight of carbonaceous material is effective with the more preferred amount being between about 25 and 150 parts by weight, and depending on the kinds and amounts of phenolic compounds employed, the preparation of the carbonaceous material and the conditions selected, the most preferred amount is about 50 parts. The amount of water in stream (4) should preferably be sufficient to maintain the alkaline material in the ionic form in solution at the herein described ionic liquefaction conditions, and sufficient to allow the water gas shift reaction (equation XI), to produce the hydrogen required for solvent regeneration and ionic species stabilization in the hydrogenation (E) step. The amount of water in water-alkali mixture stream (4) is between about 25 and 400 parts by weight, more preferably between about 50 and 250 parts by weight, and most preferably between about 100 and 200 parts by weight. Make-up alkali may be provided to stream (4) via a make-up alkali stream (4A).

The liquefaction section (B) is presented in more detail in Fig. 2. A high pressure slurry pump (K) can be used to pump the slurry, stream (5) from the preparation section (A) of Fig. 1 and to bring the slurry to the desired system pressure. The slurry then passes through the slurry-hot product heat exchanger (L) to provide initial slurry heating through waste heat recovery from the product slurry stream in the separation section (C) of Fig. 1. The slurry is then mixed with high pressure synthesis gas, stream (6), from the gasification/gas processing section, sections (G) and (H) of Fig. 1.

If synthesis gas is used, the composition of the synthesis gas stream should primarily be composed of carbon monoxide and hydrogen, although small amounts of impurities such as nitrogen and carbon dioxide can be present and still achieve the most preferred results. The preferred H₂/CO ratio under the conditions described is between about 0.5 and 2.0; a more preferred ratio is between about 0.5 and 1.5; and the most preferred ratio is between about 0.75 and 1.25. Other concentrations under different reaction conditions may also be effective.

Preferred gas treatment rates are between about 1.25 m³/kg carbonaceous material and 0.16 m³/kg (40,000 SCF/ton to 5,000 SCF/ton), the most preferred gas treatment rates are between about 0.47 and 0.16 m'/kg (15,000 to 5,000 SCF/ton).

Referring to Fig. 2, the reaction mixture, stream (26), is then brought to the desired temperature in a gas-fired tube heater (M), operated under turbulent flow conditions to optimize heat transfer. Process derived low or medium calorific value gas from gas processing sections (H) and (I), lines HF and IF, is used to fire the preheater. The reaction mixture stream (27), is then transferred to the liquefaction reaction (N) and held at the desired reaction temperature long enough for the initial ionic liquefaction process steps to take place to the desired extent. The solubilization and ionic reaction steps, but not the solvent regeneration or ionic species upgrading, take place in this reactor. The preferred reactor design is a high length to diameter ratio reactor with internal baffles to provide sufficient mixing of the polar solvent, alkali, and carbonaceous materials for the reaction mechanisms to proceed efficiently. Depending upon the desired product distribution, and desired reactant residence time distribution, other reactor designs can, of course, be selected for use. Temperature and pressure may be adjusted for the optimum conversion of individual carbonaceous feed materials.

Preferred reactor (N) residence times are from about 2 to about 120 minutes, and most preferably from about 15 to 45 minutes depending on reactor design. The preferred temperature range is from about 250°C to 350°C. (482°F to 662°F). It is important that a system pressure is selected and maintained at such a predetermined level which will keep sufficient water in the liquid phase to maintain ionic alkaline species in the liquid phase, rather than as salts, during a substantial portion of the reaction time. The preferred pressure range is between about 3.45 MPa to 17.24 MPa (500 psia to 2500 psia), and the most preferred pressure range is about 5.52 MPa to 8.28 MPa (800 psia to 1200 psia) for achieving the foregoing liquid phase.

The reaction products exiting reactor (N), stream (7) of Figs. 1 and 2, are then separated into component streams in the separation system, section (C) of Fig. 1. A more detailed schematic of this system is shown by Fig. 3. The reaction products stream (7) is fed to gas-slurry separator(s). The gas-slurry separator(s) serve to separate the majority of the slurry product from gaseous products. The separator pressure is maintained at a lesser or reduced pressure than the liquefaction reactor, preferably between about 0.69 and 3.45 MPa (100-500 psia), and the temperature is kept at conditions sufficient to keep most of the volatile organic compounds in the liquid phase, but much of the remaining water as vapor. The preferred temperature range is 200 to 300°C (392 to 572°F); the most preferred temperature range is 200 to 250°C (392 to 482°F). The slurry phase residence time is preferably less than 30 minutes, more preferably less than 15 minutes, and most preferably less than 5 minutes.

The vapor, stream (28), from the gas-slurry separator is passed to a water condenser (P) where the majority of the water is condensed, along with residual organic compounds, such as polar solvents and (C₄+) hydrocarbons. Typical concentrations of water vapor in the gas phase entering the condenser will be between about 25 to 45 mole percent and leaving the water condenser the water vapor in the gas phase will have been reduced to between about 0.01 and 0.05 mole percent. The other components of the gas stream are typically carbon monoxide, carbon dioxide, C₁ th.rough C₃ hydrocarbons, COS, H₂S, NH₃ and possibly small amounts of other gases, such as nitrogen. The preferred H₂/CO ratio'of this gas stream should generally be greater than about 2 to 1, and most preferably greater than about to 1. The water rich stream, stream (31), from the condenser (P) is preferably withdrawn through, stream (33), from the separation system, and may be used for plant cooling water or the like. However, water may be added back to the slurry from the gas-slurry separator (stream 32), if needed, to improve the slurry filtration characteristics. The slurry stream (24), goes to the feed slurry-hot product heat exchanger (K), then through a pressure let- down valve and through stream (30), to the filtration apparatus (Q).

Leaf filters, candle filters, centrifuges, hydroclones, or comparable equipment can be used for the filtration. Solids may also be separated by processes such as solvent deashing, or critical solvent extraction. The purpose of the filtration step is to separate unreacted carbonaceous material and alkaline salts from the ionic liquefaction product liquids. Due to the hygroscopic nature of the alkaline salts, much of the water present will also be separated with the filter cake.

The preferred temperature for filtration is preferably between about 150 and 100°C (302 and 212°F). The pressure is maintained at a sufficient level to obtain efficient filtration, preferably between about 0;34 and 1.03 MPa (50 psia to 150 psia). In the filtration step, the solids content of the liquid is typically reduced to less than about 1.0 percent by weight, the mineral matter content to less than about 0.5 percent by weight, and the alkaline species content to less than about 0.25 percent by weight. The values obtained are dependent upon factors such as the degree of comminution used in feed preparation, the ionic liquefaction conditions selected, and the design of the filter equipment design. The separation train should preferably be operated to reduce the alkaline compound content of the filtrate stream (10) of Fig. 1 below about 0.25 percent by weight, more preferably below about 0.15 percent by weight, and most preferably below about 0.10 percent by weight. Alkaline compound concentrations above this level are not desirable since that can lead to coking problems, and to unwanted organic ionic compound precipitation in downstream processing steps. Liquids, stream (10) of Fig. 1, with alkaline compound contents of about 0.25 percent by weight and lower may successfully be further processed by distillation (D) and hydrogenation (E), although the upper limit is dependent upon the exact nature of the product. The solids rich filter cake, stream 8 is used as feed to a gasification system (G) for production of synthesis gas and recovery of alkaline compounds (J). The gas stream, stream (9B) of Fig. 1, is sent to gas processing (1) for upgrading before use as hydrogen rich gas in subsequent hydrogenation (E) operations.

The liquids from the separation system are sent, stream (10) of Fig. 1, to a distillation tower (D) where the crude ionic liquefaction product is fractionally distilled. The products from the distillation are water, stream (11) of Fig. 1, a recycle solvent stream, stream (2) of Fig. 1, and a crude product, stream (12) of Fig. 1. A schematic of a typical distillation column is given in Fig. 4.

The distillation operation has three primary purposes. First, excess water is removed from the crude product stream. Second, a polar recycle solvent stream containing greater than about 50 weight percent phenolic materials is recovered. Third, a concentrated ionic compound stream is produced.

The production of the concentrated crude stream serves to reduce the size of downstream stabilization operation. This operation is typically accomplished by taking a 200°C (392°F) cut of the incoming feed. The distillation column is typically operated at or near atmospheric pressure preferably at about 0.10-0.15 MPa (14.5-21.75 psia). The condenser is operated as a partial condenser to separate the overhead product into an organic rich liquid phase and a water rich vapor phase. Using typical ionic liquefaction feed ratio of about 2 parts solvent to 1 part carbonaceous feed, in stream (5) of Fig. 1, the overheads to bottom ratio will be about 1 to 1, although the exact value will vary depending on the bottoms viscosity desired.

The physical properties of the distillation feed and bottoms streams are a function of the carbonaceous feed and the ionic liquefaction conditions. In a process using a feed comparable to a Texas lignite and about a 2 to 1 solvent to feed ratio, the preferred viscosity of the distillate feed is between about 1 x 10-₅ and 1 x 10⁻⁴ m²/s at 38°C (10 and 100 centistokes at 100°F). The preferred density of this stream is between about 1000 and 1200 kg/m³ (1.0 and 1.2 grams/ml).

The overheads organic liquid preferred viscosity is between about 5 x 10-⁶ and 2 x 10-⁵ m²/s at 38°C (5 to 20 centistokes at 100°F). The preferred density of this stream may be between about 950 and 1100 mg/m³ (0.95 and 1.1 grams/ml).

The preferred viscosity of the crude is between about 5 x 10-⁴ and 2 x 10-³ m²/s at 38°C (500 and 2000 centistokes at 100°F). The preferred density of the crude is between 1100 and 1200 kg/m³ (1.1 and 1.2 grams/ ml). The crude will normally contain at least about 40% phenolic compounds.

Three processes may be used in the ionic liquefaction process described to upgrade the resultant crude. The first embodiment, shown in Fig. 1, is hydrogenation. Alternatively, the crude may be stabilized by acid hydrolysis or by coking. A schematic of a typical hydrogenation and distillation train is shown in Fig. 5, a schematic of a typical acid hydrolysis train is shown in Fig. 6, and a schematic of a typical process incorporating coking is shown in Fig. 9.

Referring to the process schematic shown in Fig. 5, the hydrogenation train may consist of four major processing units: (1) crude preheaters (R) and (S'), (2) a crude hydrogenation reactor (T), (3) a gas-oil phase separator (U), and (4) a catalyst regeneration-alkali recovery unit (V).

The incoming crude stream (12), is first preheated in a waste heat recovery preheater (R) through heat exchange with the refined crude oil, stream (17) from the gas separator. The remainder of the heating is accomplished in a gas-fired tube heater (S'). The preheated crude stream is then passed to the hydrogenation reactor (T) where it is reacted with a hydrogen-containing gas which is introduced into the hydrogenation reactor (T) as stream 13. The preferred operating condition for the hydrogenation reactor (T) is in a slurry phase catalytic hydrogenation mode. The preferred operating conditions permit separation of the refined crude and catalyst using a solids disengaging zone, and a catalyst withdrawal operation. Preferred hydrogenation conditions are those which are severe enough to break ether bonds and upgrade ionic species, but which are not severe enough to favor saturation of aromatic rings or the removal of organic oxygen as water. Preferred operating temperature is between about 343 and 454°C (650 and 850°F, and most preferably between about 343 and 400°C (650 and 752°F). The preferred pressure range is between about 6.9 and 13.8 MPa (1000 and 2000 psia). The preferred catalyst types are standard hydrogenation catalysts such as Co-Mo/A1₂0₃ and Ni-Mo/AI₂O_{3,} typically about 1/32, 1/16 or 1/8 inch extrudate form. Preferred catalyst loadings are about 0.01 to 1.0 kg cat/kg oil/hr, more preferred loadings are about 0.01 to 0.5 kg cat/kg oil/hr, the most preferred loadings are about 0.05 to 0.15 kg cat/kg oil/hr. Preferred hydrogen treatment rates are about 178 to 1424 m³H₂/m³ oil (1000 to 8000 SCFH₂/BBI oil); more preferred hydrogen treatment rates are about 178 to 712 m³H₂/m³ oil (1000 to 4000 SCFHJBBI oil. Preferred hydrogen consumption is less than about 3.90 kg HJm3 oil (1.36 Ib H₂/BBI oil), and more preferably less than about 1.94 kg H₂/m³ oil (0.68 ib H₂/BBI oil). It is desirable to hold the crude at the temperature selected for sufficient time to permit the solvent regeneration and ionic stabilization reactions to occur. Preferred residence times are between about 10 and 90 minutes, more preferably between about 15 and 60 minutes, and most preferably between about 30 and 45 minutes.

In the catalyst regeneration-alkali recovery unit (V) the catalyst rich slurry is first degassed, and the gases, stream (42), mixed with other exit gases, stream (39), from the hydrogenation train, and passed via stream (18) to gas processing unit (I). The catalyst and refined oil are separated by standard solid-liquid separation devices such as filters or hydroclones. Residual refined oil and soluble alkali salts are recovered by hot water leach. The leachate is recycled to the liquefaction reactor, unit (B) of Fig.1. Coke is burnt off the catalyst by fluid bed combustion in the presence of added air or oxygen, spent catalyst is removed, stream (15), makeup catalyst is added, stream (41 B) and the regenerated catalyst, stream (16), is recycled to the hydrogenation reactor (T) (Fig. 5).

Refined ionic liquids in stream (17) are separated from the treatment gases in a gas liquid separator (U). The gases in stream (39), are sent to gas processing for upgrading by removal of acid gases and light hydrocarbons.

The refined liquids from the hydrogenation train, depending on the conditions employed, will preferably have been converted to greater than 80 wt percent oils, more preferably than 90 wt percent oils, and most preferably greater than 95 wt percent oils, as defined by pentane solubility and ASTM D1160-77 distillation results. The preferred viscosity of the refined oil is between about 5 x 10-⁶ and about 1 x 10-⁴ m²/s at 38°C (5 to 100 centistokes at 100°F), and more preferably between about 5 x 10-⁶ and 2 x 10-⁵ m²/s (5 to 20 centistokes at 100°F). The preferred density of the refined oil is between about 1000 and 1100 kg/m³ (1.0 to 1.1 grams/ml). The refined oils, stream (17) of Fig. 1 and stream (38) from catalyst regeneration alkali recovery unit (V), are then sent to a distillation unit, unit (F) for final processing as will be described in detail hereinafter.

The second upgrading embodiment is acid hydrolysis, as shown in Fig. 6. In this process alternative, hydrogen is added to the ionic organic species in the crude through ionic reactions with acid. In one method, carbonic acid produced in the acid hydrolysis train is used as the hydrogen source, although small amounts of other acids alone or in combinations can be used, such as sulfuric acid, hydrochloric acid, formic acid, acetic acid, and carbamic acid, which will enhance the rate and extent of ionic hydrogenation.

Referring to Fig. 6, the acid hydrolysis train consists of five units, (1) a gas absorber tower (AA) to produce carbonic acid, (2) a crude stabilizer (BB), (3) a liquid phase separator (CC), (4) a high-oxygen product distillation tower (DD), and (5) low-oxygen product distillation tower (EE).

In the preferred operation, carbonic acid is produced through gas absorption in a counter-current gas absorber (AA). Water is fed in, stream (101) at the top of gas absorber tower (AA), and carbon dioxide or carbon-dioxide rich gas from the ionic liquefaction reactor or other source is fed in the bottom of the gas absorber tower (AA) stream (98). The absorber is operated in such a manner to produce carbonic acid, stream (103), with a concentration preferably between 1650 mole/m' (0.103 Ib. mole/ft³) and 40 mole/m³, more preferably between 1650 molelm³ and 1000 molef, which is passed to crude product stabilizer (BB). The absorber is preferably operated in the temperature range 16 to 66°C (60 to 150°F), and more preferably in the range 16 to 32°C (60 to 90°F). The preferred operating pressure is in the range of about 0.34 to 10.35 MPa (50 to 1500 psia), and more preferably in the range 6.90 to 10.35 MPa (1000 to 1500 psia). The tower may be operated as a bubble cap column, although other designs such as packed columns, venturi scrubbers, or spray towers may be used. Excess carbon dioxide gas is removed, stream 102, and may be recycled in known manner to qas absorber tower (AA).

The ionic acid-base reactions take place in the crude product stabilizer (BB). Stabilizer (BB) is operated in a stirred tank mode to maximize the contact between the aqueous and organic phases. Although dependent upon the degree of stabilization required and the strength of the acid, the preferred feed ratio by volume to the stabilizer is 10 parts acid to 1 part topped crude, more preferably 5 parts acid to 1 part crude, and more preferably 1 part acid to 1 part crude. The preferred temperature is less than about 200°C (392°F), more preferably less than about 150°C (302°F), and most preferably less than about 100°C (212°F). The pressure is kept sufficiently high to keep the majority of the carbon dioxide in the liquid phase, preferably between 6.90 and 13.80 MPa (1000 and 2000 psia), and more preferably between 10.35 and 13.80 MPa (1500 and 2000 psia). The acid and crude are maintained at stabilization conditions for sufficient time to permit the desired stabilization reactions to take place. The preferred time is between about 5 and 90 minutes, and a more preferred time is between about 15 and 45 minutes.

In an alternate configuration the carbon dioxide rich gas and water are added directly to the stabilizer, eliminating the gas absorption unit. Stabilization conditions employed can remain the same.

A two phase aqueous-organic product, stream (104), is withdrawn from crude product stabilizer (BB) and is sent to a liquid separator (CC) where gravity separation is used to generate a light aqueous-rich product stream (106) and a heavy organic-rich product stream (105).

Liquid separator (CC) may be operated at ambient temperature. The preferred residence time is between about 10 and 60 minutes, and more preferably between about 10 and 30 minutes.

The light aqueous-rich stream is passed to a distillation unit (DD) where water, stream (107), an oxygen rich water soluble product stream (108), and a residual product stream (109) are recovered. Because of the normally high solubility of alkaline compounds in the water phase, the majority of residual alkaline materials will be present in the residual product from this distillation unit.

The heavy organic rich phase stream (105), is passed to a second distillation unit (EE), where various distillate products such as naphtha, stream (110), light and heavy gas oil fractions, streams (111) and (112), and a residual product stream (113) are obtained.

An alternate acid hydrolysis configuration is shown in Fig. 7, where an acid other than carbonic acid is used as the hydrogen donor species. The major processing units in this embodiment are a crude product stabilizer (FF), a liquid separator (GG) and two distillation towers, (HH) and (II).

In the crude product stabilizer the crude product stream (12) is stabilized with an acid from stream (115) at a temperature sufficient to permit the ionic stabilization reaction to proceed to the desired extent.

The preferred acid for this embodiment is sulfuric acid. A portion of the sulfuric acid could come from acid gas removal operations, unit (I) of Fig. 1. Additional required sulfuric acid would have to be added as make-up acid, stream (121).

The acid and crude are intimately contacted in a stirred tank reactor operation under acid reflux conditions that is, at the boiling point of the acid. The preferred ratio of acid to topped crude is about 10 to 1, a more preferred ratio is about 5 to 1, and the most preferred ratio is about 1 to 1. The temperature of the system will be predominantly governed by the boiling point of the acid solution which is preferably between about 204 and 100°C (400 and 212°F), more preferably between about 149 and 100°C (300 and 212°F), and most preferably between about 120 and 100°C (248 and 212°F). The pressure is preferably maintained at about atmospheric pressure. The residence time in the crude product stabilizer is preferably between about 5 and 90 minutes, and more preferably between 15 and 45 minutes.

The two-phase aqueous-organic product in the stream (114) is then sent to the liquid separator (GG) where gravity separation is used to generate a light aqueous-rich product in a stream (116), and a heavy organic-rich product in a stream (117). The preferred residence time is between 10 and 60 minutes and more preferably between 10 and 30 minutes.

The light aqueous-rich stream (116) leaving the liquid separator is divided into two streams (118 and 120). Stream (120) is mixed with make-up acid (121) and recycled to the crude product stabilizer (FF). As noted supra, make-up acid can come from the acid-gas removal unit in the gas processing unit, (I) of Fig. 1, and from purchased acid. The remaining aqueous liquids in the stream (118) are sent to a distillation tower (II) where water is vaporized, and transferred in stream (119) for recycling to the crude product stabilizer (FF). An organic distillate, stream (126) and a spent acid stream, stream (127) consisting of heavy organics and alkaline salts such as Na₂SO₄ are also produced.

The organic rich phase in stream (117) is passed to a second distillation unit (HH) where various distillate products such as naphtha, stream (122), light and heavy gas oil, fractions, streams (123) and (124) and residuum, stream (125) are obtained.

Fig. 8 presents a modified schematic of the integrated ionic liquefaction process using acidification in an acidification unit (FF) for the ionic liquid stabilization, and acid recovery in an acid recovery unit (AR).

A third upgrading embodiment is coking as shown in Fig. 9. In this processing option the crude stream (12), from distillation tower (D) is further upgraded in a delayed or fluid bed coking operation (KK), which coke, stream (K1) being produced, and water, stream (K2) being removed.

Coking is defined as a severe thermal cracking process in which one of the end products is a carbon rich solid, i.e. coke, the other products are hydrocarbon gases, and ligands.

In the present invention, the coking operation will proceed at about atmosphereic pressure and at temperatures from about 427°C (800°F) to 510°C (950°F).

Using 1000 parts of crude as an example, the coking operation may produce from about 250 to 300 parts coke, from about 80 to 120 parts (C₄) hydrocarbons, from about 300 to 50 parts water, and the remainder as liquids. The liquids produced will be used as recycle solvent. The gases will be sent, stream (131) to gas processing.

Support equipment and facilities for ionic liquefaction can be commercially obtained and include gasification and various gas processing operations. such as compression, acid gas removal, and shift conversion processing to increase hydrogen content of gas streams. The actual configuration is dependent upon the type of stabilization operation used, that is hydrogenation, acid hydrolysis, or coking.

Referring to the integrated process using hydrogenation for stabilization, Fig. 1, the filter cake produced in the separation operation, unit (C), is used as a feed stream (8), to a gasifier, unit (GH). In the configuration shown in Fig. 1 the preferred gasification operation is a dry ash partial combustion process to produce a synthesis gas rich in carbon monoxide and hydrogen. The preferred H₂/CO ratio of gas leaving the gasifier, stream (22), is between 0.5 and 2.0. Acid gases and light hydrocarbon gases are separated from the synthesis gas by standard operations in gas processing operations, unit (H).

The ash from the gasifier, stream (21) is sent to an alkali recovery unit (J) where the majority of the alkaline compounds are separated from the ash stream by hot water extraction, and recycled, stream (4), to the preparation unit (A), and the residual ash removed, via stream (J1). The expected recovery of alkaline compounds is greater than 50%, and can be greater than 75%, and even greater than 90%. The preferred temperature is between 25 and 100°C (77 and 212°F), and more preferably between 50 and 100°C (122 and 212°F). The preferred treatment rate is less than 4 kg H₂0/kg ash, more preferably less than 2 kg H₂0/kg ash, and most preferably less than 1.1 kg H₂0/kg ash.

In an alternate configuration alkaline compounds may be removed from the feed, stream (8), to the gasifier (G). The preferred processing conditions remain as before.

For hydrogenation (Fig. 1) the gas processing unit (I) consists of a conventional shift converter for producing a hydrogen rich gas, stream (13), for hydrogenation at hydrogenation unit (E), and acid gas, stream (IW), removal operations to remove C0₂ and sulfur containing gases.

In acid hydrolysis (Fig. 8) this gas processing operation consists of acid gas removal operations, where the sulfur removal operation produces sulfuric acid, stream (lA), and/or CO₂, stream (IB), for use in the acid hydrolysis operation.

In the coking operation the gas processing operation may consist of acid gas removal operations to produce a high calorific gas for plant fuel and for sale.

The following Examples demonstrate the kinds of results that are obtainable with the feeds and conditions cited.

### Example 1

A series of experiments were performed to model the integrated ionic liquefaction process from slurry mixing to hydrogenation. All experiments were performed in a single pass batch mode.

The experiments were performed in a semi-batch liquefaction system. The major components of the system are the gas delivery system, reactor system and gas measurement system. The gas delivery system consists of a Whitey gas compressor. The primary components of the reactor system is a 0.001 m³ (1.0 liter) magnedrive Autoclave manufactured by Autoclave Engineers. A knock-back condenser is used to minimize liquid loss from the reactor. System pressure is maintained using a Grove dome-loaded back-pressure regulator. The gas measurement systems consist of a Rockwell diaphragm meter for total gas volume, and a Carle Series S chromatograph for on-line analysis of water gas shift components, light hydrocarbons and Argon tracer.

To produce sufficient material for all steps for the process, a series of four identical experiments were performed. Conditions for these experiments are listed in Table 1. The Texas Lignite used in these experiments was obtained from a single large parent coal sample. At the completion of each run, the reactor product was removed and filtered. Samples were removed from the reactor product of the last run for selective solvent extraction analysis. The procedure is an empirical method to determine the quality of the product. Ten grams of the reactor product is extracted with three 150 ml washes of tetrahydrofuran (THF) in centrifuge bottles. Each wash is centrifuged and the liquid decanted. The solids are dried and weighed. The THF insoluble material correspond to unreacted carbonaceous material. The THF soluble fraction is rotovaped and the THF removed. The remaining liquid is washed with toluene in the same manner as the THF. The toluene insoluble solids correspond to high molecular weight material. The toluene soluble material is rotovaped and washed with pentane in the same manner as the THF. The pentane insoluble material is lower molecular weight material and some polar material. The pentane soluble material corresponds to oils or low boiling (760°F) compounds. The MAF (moisture and ash free) and DMMF (dry mineral matter free) yield structure was:

The filter cakes were collected and analyzed for moisture, ash, and sodium content. The filtrate from each run was individually distilled to remove one half of the material (by weight). The overheads of each run were collected and mixed together. The bottoms were also collected and mixed together. A summary of the material balance for these experiments is shown in Table 2. The data indicate that over 80% of the MAF coal is converted to a liquid product (81.1% calculated from cake weight, 85.6% calculated from filtrate weight). This step also indicates that 85.6% of the MAF coal can be separated by filtration for the distillation.

A sample of the bottoms was upgraded and stabilized in a hydrogenation experiment. The bottoms (494 grams), Harshaw Catalyst 601-T (50 g), and Na2S.9H20 (25 g) were mixed together in the reactor. The Harshaw catalyst is a Cobolt-Molybdenum catalyst. The Na₂S was added to increase the activity of the catalyst. The hydrogenation experiment was performed at 400°C (725°F) for a period of 60 minutes at temperature. A system pressure of 13.90 MPa (2012 psia) was maintained with gas flow of 5 x 10-⁵ m³/s. A 95:5 mixture of hydrogen and argon was used as the gas.

At the completion of the experimental run the reactor product was centrifuged and the decants collected. The bottoms were mixed and analyzed for moisture, ash, ash components, and by SSE. The decant was analyzed by SSE to determine pentane soluble yields.

The physical properties of the topped crude were greatly changed by hydrogenation, as shown in Table 3. Solvent extraction showed that all the THF insoluble material was in the decant bottoms. Overall there was a 55% reduction in the THF insolubles, a 100% reduction in the toluene insolubles, a 65% reduction in pentane insolubles and a 56% increase in the pentane soluble. For the ionic liquefaction process this would result in 25.7 kg (56.5 Ib) of Pentane Solubles for every 45.5 kg (100 pound) MAF coal.

The gas stream from the reactor was analyzed for gas production and for the quantity of hydrogen consumed. The gas analysis showed that there was 1.7 g-mole of hydrogen consumed which corresponds to 1.4 wt% of the MAF coal fed.

### Example II

A suite of six coals were experimentally tested to determine suitability as ionic liquefaction feedstocks. The coals ranged in rank from an Australian brown coal to a high volatile B bituminous. Analyses of the suite coals are given in Table 4.

Experiments were performed at the conditons noted in Table 2, except for the experiments using the Australian brown coal which were performed at lower temperature because of the high moisture content of the coal.

In general all of the coals tested to give satisfactory yields as shown in Table 5 although the lower rank coals seem to be more suitable ionic liquefaction feedstocks because of large oil and gas yields.

An alternative process has been developed to solvate carbonaceous material with a solvent/solute system, to filter the solid ash and undissolved organic material from the liquid, and to distill a recycle solvent fraction leaving behind a solid with reduced sulfur and ash content. The solid product formed can be used as a clean burning boiler fuel as a replacement for oil or coal. Use of this product has economic advantages over oil and eliminatesd many of the environmental problems associated with the burning of coal, such as sulfur emissions and ash handling problems. This is accomplished with a solution of phenols, alkali, and water mixed with the carbonaceous material. The slurry is heated with or without the presence of gas or any gas partial pressure.

The slurry is heated in the range (300°C to 360°C) for a period of from 60 minutes to 90 minutes. The pressure of the system is that exerted by the liquids present in the system at the temperatures employed, which will typically be in the range of from 2.07 to 10.35 MPa (300 to 1500 psia).

After solvation of the carbonaceous material in an ionic liquefaction reactor the slurry is removed and the temperature and pressure reduced. The slurry is filtered to remove the ash and undissolved organic material that has not dissolved and in the solvent/solute system. A large portion of the ash will be removed in this step including a majority of the inorganic sulfur. The filtrate is then transferred to a liquid extraction stream to remove dissolved ash components and alkali. The ash and alkali are removed by contacting the filtrate with an acid such as carbonic (H₂C0₃), HCI, H₂SO₄ or the like. Dissolved inorganic compounds will be removed because of their great affinity for the aqueous layer as opposed to the organic filtrate. The acid will replace alkali atoms present as alkali-organic salts with hydrogen with the alkali being soluble in the aqueous layer. The liquid extraction stream will include a final water wash of the filtrate to remove any remaining inorganic constituents as well as acid components still present in the organic layer.

The extracted and washed filtrate is then distilled to recover the solvent. The overheads from the distillation tower are used as recycle solvent. The distillation temperature is raised sufficiently to remove the fraction boiling under about 275°C, more preferably under about 300°C and more preferably under 325°C. The bottoms from the distillation are collected and cooled to form a solid product which has reduced sulfur and ash.

Sulfur can be removed in a variety of ways. The inorganic fraction which is mainly pyrite, will be removed as an insoluble material in the filtration step after the solvation of the carbonaceous material. Organic sulfur is removed by reaction with alkali and base to form such compounds as alkali sulfides, sulfites, and sulfates. The resulting sulfur compounds are either removed during the filtration step or during the acid extraction of the filtrate depending on the solubility of the species. A sulfur scavenger may also be added to the ionic liquefaction step which is selected to react with sulfur compounds to form insoluble species.

Referring to the schematic diagram in Fig. 10, a process is shown which favors the production of a' product which is solid at room temperature and is useful as a fuel substitute. The feed preparation at (A1), as previously described, comminutes the carbonaceous material (stream 100) by conventional means, as previously described; and adds a water-alkali mixture, stream (300); and recycle polar solvent, stream (200) containing greater than 50% by weight of phenolic species. The comminution process may again be accomplished either dry or wet. If performed wet, then the recycle polar solvent may be used as the wetting agent. The carbonaceous feed is, as before, comminuted to 100 percent minus 74 microns (200 mesh) particle size, more preferably to 100 percent minus 147 microns (100 mesh) particle size, and most preferably to 100 percent minus 350 microns (40 mesh) particle size but in any event must be in a form which will enable the requisite solubilization for the ionic liquefaction to proceed.

Using 1000 parts by weight of the stream of carbonaceous material introduced into the feed preparation at (A1) as an example, the preferred amount of polar recycle solvent for the required solubilization to proceed, introduced by stream (200) is between 1500 and 3500 parts by weight depending on the prepared form of the carbonaceous material, with 3000 parts by weight of solvent the most preferred amount. The polar recycle solvent contains preferably greater than about 50% by weight phenolic compounds, and more preferably greater than 60% by weight phenolic compounds.

The preferred amount of alkaline material in stream (300) is selected to be that amount which is to produce the desired results. It has been found under the conditions disclosed herein that between about 25 parts and 400 parts by weight is effective with the more preferred amount being between about 25 and 150 parts by weight, and depending on the kinds and amounts of phenolic materials employed, the preparation of the carbonaceous material and the conditions selected, the most preferred amount is about 50 parts. The amount of water in stream (300) should preferably be sufficient to maintain the alkaline material in the ionic form in solution at the described ionic liquefaction conditions. The amount of water in stream (300) is between about 25 and 400 parts by weight, more preferably between about 50 and 250 parts by weight, and most preferably between about 100 and 200 parts by weight. Make up alkali, (stream 300A) may be added, as before.

The liquefaction section (B1) is the same or similar to that shown in (B) Fig. 1. A high pressure slurry pump (not shown) can be used to pump the slurry, stream (400) and to bring the slurry to the desired system pressure. The slurry at this point may or may not have a synthesis gas added. The reactions can proceed without the added gas. If added gas is used, the gas is introduced before further processing.

The composition of the synthesis gas stream can be as previously described.

Preferred gas treatment rates are also as previously described.

The reaction mixture is then brought to the desired temperature. The reaction mixture stream is then transferred to the liquefaction reactor (B1) and held at the desired reaction temperature for sufficient time to permit the ionic liquefaction process steps to take place to the desired extent. The solubilization and ionic reaction steps, but not the solvent regeneration or ion species upgrading, take place in this reaction. Temperature and pressure should be optimized for individual carbonaceous feeds.

Preferred reactor residence times are from 2 to about 120 minutes, and most preferably from about 15 to 45 minutes depending on reactor design. The preferred temperature range is from about 250°C to 360°C (482°F to 680°F). System pressure should be established and maintained at such a predetermined level so as to keep sufficient water in the liquid phase to maintain ionic alkaline species in the liquid phase, rather than as salts, for a predetermined portion of the reaction. The preferred pressure range is from about 0.69 MPa to 13.80 MPa (100 psia to 2000 psia), and the most preferred pressure range is about 2.76 MPa to 88.2 MPa (400 psia to 1200 psia).

The reaction products leaving the reactor (B1), in stream (606) of Figs. 9 and 10, are then separated into component streams in the separation system, process (C1) of Fig. 10. The gas-slurry separators employed serve to separate the majority of the slurry product from gaseous products. The separator pressure is maintained at reduced pressure, preferably between about 0.69 and 3.45 MPa (100-500 psia), and the temperature is kept at conditions sufficient to keep most of the volatile organic compounds in the liquid phase, but much of the remaining water as vapor. The preferred temperature range is 200 to 300°C (392 to 572°F); the most preferred temperature range is 200 to 250°C (392 to 482°F). The slurry phase residence time is preferably less than 30 minutes, more preferably less than 15 minutes, and most preferably less than 5 minutes.

The vapor stream (601) from the gas-slurry separator goes to a carbon dioxide separation step (E1) then to sulfur recovery (K1) for separation into a flue gas stream (FG) and a sulfur stream (S1).

As previously described, leaf filters, candle filters, hydrociones, or comparable equipment can be used for the separation of the solids as well as separation by processes such as solvent deashing, or critical solvent extraction. The purpose of the filtration is to separate undissolved carbonaceous material, ash and alkaline salts from the ionic liquefaction products which are liquid under the conditions employed. Due to the hygroscopic nature of the alkaline salts, much of the water present will also be separated with the filter cake.

The preferred temperature for the separation step (C1) is preferably between about 150 and 100°C (302 and 212°F). The pressure is maintained at a sufficient level to obtain efficient separation, preferably between about 0.34 and 1.03 MPa (50 to 150 psia). In the separation step, the solids content of the liquid in the stream (609) is typically reduced to less than about 1.0 percent by weight, the mineral matter content to less than about 0.5 percent by weight, and the alkaline species content to less than about 0.25 percent by weight. The values obtained are dependent upon factors such as the degree of comminution used in the feed preparation, ionic liquefaction conditions, and filter equipment design. The separation train should preferably be operated to reduce the alkaline compound content of the stream (609), of Fig. 10, below about 0.25 percent by weight, and most preferably below about 0.15 percent by weight, and most preferably below about 0.10 percent by weight. The liquid stream (609) of Fig. 10 with alkaline content less than .25 percent will have the alkaline content reduced further by washing in a solvent extractor system, such as shown in Fig. 11. The liquid stream (609) is contacted with the solution stream (610) of Fig. 10 containing added fresh water in a countercurrent method while bubbling C0₂, steam (611) through the solution in a mixing vessel (M1) as shown in Fig. 11. The resulting liquids stream (615) is passed to a liquid/liquid settler (S1) for separating the liquids stream into an organic component and an aqueous component. The organic component stream (613) of Fig. 11 will have the alkaline and ash concentration reduced less than 0.05%, more preferably to less than .02% and most preferably to less than .005%. In the preferred embodiment of the process, the liquid stream (609) and water stream (610) are contacted in mixing vessel (M1) in a feed ratio of one part filtrate (609) to 5 parts H₂0, more preferably one part feed to 3 parts H₂0, and most preferably one part feed to one part H₂0. The preferred temperature is about 100°C (212°F), more preferably less than about 80°C (176°F) and most preferably less than about 50°C (122°F). The liquid streams and CO₂ will preferably be mixed for a period of 15 minutes, and more preferably for a period of between 5 and 10 minutes. The carbon dioxide when bubbled through the aqueous solution produces carbonic acid which replaces the alkali in the organic solution with hydrogen. An organic-rich stream (613) is separated in separator (S1) and sent to a distillation unit (11) (Fig. 10) where the organic rich stream is fractionally distilled. A light oil fraction is collected as a product stream (626). Distillate product boiling between 200°C and 325°C (392°F and 617°F) is collected as a recycle solvent stream (200) and returned to the feed preparation (A1). The high boiling fraction is collected and cooled to about 25°C. This is a product stream (627), which at room temperature, is a pseudo-plastic solid with an ash content below 1 %, more preferably below 0.3%, and a sulfur content below 1.0%, more preferably below 0.5%, and most preferably below 0.3%. The solids rich filter cake (607) is washed with a water stream at solids washing unit (F1). The water stream is preferably at a temperature of 80°C and at a ratio to the coke of 5 to 1, preferably 3 to 1, and most preferably 1 to 1. The water stream will remove liquid organics associated with the filter cake and the water- organic stream (610) and is sent to the solvent extraction system (D1).

Referring further to the integrated process in Fig. 10, the washed filter cake produced in the solids washing unit (F1), is used as a feed stream (614), to a gasifier, unit (G1). In the configuration shown in Fig. 10 the preferred gasification operation is a dry ash partial combustion process to produce a synthetic gas rich in carbon monoxide and hydrogen. The preferred H_{:}!CO ration of gas leaving the gasifier, stream (615) is between 0.5 and 2.0. Acid gases and light hydrocarbon gases are separated from the synthesis gas by standard operations in gas processing operations, unit (H1).

The ash from the gasifier, stream (616), is sent to an alkali recovery unit (J1) where a portion of the alkaline compounds are separated from the ash stream by hot water extraction, and recycled, stream (300), to the preparation unit (A1), and the residual ash removed, stream (628). The preferred recovery of alkaline compounds is greater than 50 percent by weight, more preferably greater than 75 percent by weight and most preferably greater than 90 percent by weight. The preferred temperature of the hot water used for the extraction is between 25 and 100°C (77 to 212°F), and more preferably between 50 and 100°C (122 and 212°F). The preferred treatment rate is less than 4 kg H₂0/kg ash, more preferably less than 2 kg H₂0/kg ash, and most preferably less than 1.1 kg H₂0/kg ash.

### Example III

A series of experiments were performed to model the ionic liqufaction process for the production of a solid product. The experiments were performed in a single pass batch mode modeling all process steps from slurry mixing to recovery of solid product. The liquefaction step was performed in the system described in Example I.

The experiments were performed using several types of carbonaceous feedstocks. An analysis of each feedstock is presented in Table 6. The ionic liquefaction conditions for each feedstock are listed in Table 7. The product from the ionic liquefaction reactor for each experiment was removed from the reactor. This product was filtered to remove ash and unreacted carbonaceous material. The filter cake was weighed and then washed with 180°F water to remove excess liquid product. The washed filter cake was dried and the weight recorded.

Alkali and ash material were removed from the filtrate by extraction with a 10% hydrochloric acid solution. The extractions were performed in a separatory funnel by mixing the filtrate three separate times with fresh acid solution and collecting the filtrate (organic fraction). The extracted filtrate was distilled to remove the material boiling below 300°C. The bottoms from this distillation was the solid product and was collected. Any distillate collected in excess of the solvent was coal-derived distillate and recoverable as a liquid product stream. Results from this series of experiments are presented in Table 8.

These data indicate that the process yields a solid product with greatly reduced ash and sulfur content and an increased heating value.

### txampie iv

A suite of coals have been examined to determine their suitability as feedstocks to produce a solid product from the ionic liquefaction process. Analysis of the suite of coals appears in Table 9. The experiments were performed as described in Example 3 under the ionic liquefaction conditions presented in Table 10.

In general, all of the coals tested give satisfactory yields, and produce a product with reduced sulfur and ash content. Results appear in Table 11.

### Example V

An experiment was performed using a Texas lignite. Anaylses and reaction conditions of the experiment appear in Table 9 and 10. The experiments were performed as described in Example 3 except a different extraction procedure was used. In this example the filtrate was mixed with water (1:1.5) and stirred. Carbon dioxide gas was bubbled throught the agitated solution for a period of one hour. After one hour the organic fraction was removed in a separatory funnel and distilled. The results of experiments are given in Table 11.

### Example VI

A hvBb coal obtained from the Ohio No. 6 Seam is preprocessed in a conventional gravity separation screening and drying process, and is pulverized to a top size of about -200 mesh (-74 microns). A semi-batch liquefaction unit comprising a gas delivery system, a reactor system, and a gas measurement system is charged with 100 g. of pulverised coal and 360 g. of m-cresol. The semi-batch coal liquefaction unit is designed for continuous flow of gas, and for batch injection of solid-liquid slurries. Gas is fed to the liquefaction unit from pressurized gas bottles which are premixed with 5% argon and 95% carbon monoxide. The gas delivery system is equipped with pressure regulators, and flow controllers to maintain 1012 psia (6.98 MPa) at 0.1263 gram moles per minute gas flow rate (of CO). The reactor system consists of a 316 stainless steel, one-liter Magnedrive Autoclave manufactured by Autoclave Engineers, Erie, Pennsylvania, and an iron-constantan thermocouple connected to an Omega Model 400A temperature indicator. The heater temperature is controlled by a Fenwall Series 5501552 temperature controller. Gas flow enters the reactor through the stirrer and exits through a knockback condensor consisting of a %-inch O.D. stainless steel tube in a water jacket. The gas measurement system consists of a Rockwell Model S-200 diaphragm meter for measurement of total gas volume, a Carle Series "S" chromatograph for analysis of carbon monoxide, carbon dioxide, hydrogen and argon tracer, and a Hewlett-Packard 3390 integrator to calculate and print the gas composition in mole percents. The semi-batch liquefaction reactor system is pressure tested at 1012 psia (6.98 MPa) with helium and then the premixed argon and carbon monoxide gas is introduced and the reactor is heated to 300°C (573K). After the reactor temperature and pressure are maintained for the desired reaction time, 120 minutes in this instance, the heater jacket is removed and the autoclave is cooled using forced air convection. The solid and liquid components are removed from the reactor and mixed in a high speed blender. Samples are removed from the blender and placed in 250 ml. centrifuge tubes. The samples are subjected to an empirical selective solvent extraction procedure using tetrahydrofuran (THF), toluene, and pentane to determine total conversion, preasphaltenes, asphaltenes, and oil plus gas.

The yield and product structure are defined by:

The results of the selective solvent extraction procedure are shown in Table 12. Results of the gas analysis showed 93.52 percent carbon monoxide, 0.66 percent hydrogen and 0.3 percent carbon dioxide.

Carbon monoxide conversion is calculated from analysis, over time, of the exit gas, and plotted with temperature and the results shown in Fig. 12, wherein:
0 represents CO conversion, calculated from CO in the exit gas;
and represents CO conversion, calculated from C0₂ in the exit gas, using water gas shift storchiometry; and
A represents, CO conversion, calculated from H₂ in the exit gas, using water gas shift storchiometry.

### Example VII

The foregoing procedure is repeated using 100 g. of the hvBb Ohio No. coal, 360 g. of m-cresol, 40 g. of water, 1012 psia (6.98 MPa), 300°C (573K), of 95 percent carbon monoxide and 5 percent argon, 0.01992 gram moles per minute gas flow rate (of CO), for 120 minutes. The semi-batch liquefaction unit is charged, heated and the products analyzed as previously described. The results of the selective solvent extraction procedure are shwon in Table 12 and results of the gas analysis showed 92.45 percent carbon monoxide, 0.81 percent hydrogen, and 1.15 percent carbon dioxide.

Carbon monoxide conversion is calculated and plotted, as before, and the results shown in Fig. 13.

### Example VIII

The foregoing procedure of Example VI is repeated using 100 g. of the hvBb Ohio No. coal, 360 g. of m-cresol, 40 g. of water, 25 g. of potassium hydroxide, 1012 psia (6.98 MPa), 300°C (573K), of 95 percent carbon monoxide and 5 percent argon, 0.01992 gram moles per minute gas flow rate (of CO), for 120 minutes. The semi-batch liquefaction unit is charged, heated and the products analyzed as previously described. The results of the selective solvent extraction procedure are shown in Table 12, and results of the gas analysis showed 54.54 percent carbon monoxide, 19.44 percent hydrogen, and 21.44 percent carbon dioxide.

Carbon monoxide conversion is calculated and plotted, as before, and the results shown in Fig. 14.

### Example IX

The foregoing procedure of Example VI is repeated using 100 g. of the hvCb Colarado Wadge coa' 360 g. of a synthetic recycle solvent consisting of 270 g. of m-cresol, 60 g. of 1,2,3 tetrahydronaphthalene, 20 g. of naphthalene, and 10 g. of 1-methylnaphthalene, 40 g. of water, 1012 psia (6.98 MPa), 300°C (573K), 0.5 SLM of of 95 percent carbon monoxide and 5 percent argon, and 120 minutes. The semi-batch liquefaction unit is charged, heated and the products analyzed as previously described. The results of the selective solvent extraction procedure are shown in Table 13.

### Example X

The foregoing procedure of Example VI is repeated using 100 g. of the hvCb Colarado Wadge coal 40 g. of water, 15 g. of sodium hydroxide, and the temperature, pressure, gas composition and flow rate and residence time of Example IX. The semi-batch liquefaction unit is charged, heated and the products analyzed as previously described. The results of the selective solvent extraction procedure are shown in Table 13.

### Example XI

The foregoing procedure of Example VI is repeated except 15 g. of sodium carbonate was used replacing the 15 g. of sodium hydroxide. The semi-batch liquefaction unit is heated, charged, and the products analyzed as previously described. The results of the selective solvent extraction procedure are shown in Table 13.

The results in Tables 12 and 13 demonstrate the significantly improved results obtained by practice o" the present invention. Table 13 shows that the presence of the organic phase solubilizing agent, m-cresol. in the absence of the inorganic phase constituent as Example VI, yields a MAF conversion of 40 wt%. In the case of Example VII with the addition of water, the MAF conversion is 39 wt%, which is virtually unchangec from Example VI. In Example VIII, under operating conditions of Examples VI and VII, the synergistic effect of the alkali/alkaline-earth constituent is observed as the yield is increased to 82.52 MAF wt%. In Examples IX, X and XI, the organic phase solubility agent is a synthetic solvent which is considered to represent a recycle stream in a continuous liquefaction facility. The MAF wt% yields for Example X and XI, when compared to Example IX, show the increased synergistic effect obtained by the combination of the inorganic and organic phase constituents.

### Example XII

The foregoing procedure of Example VI is repeated using 180 g. of the hvCb Colarado Eagle No. 5 coal. The organic fraction of the solvent/solute system is 360 g. of synthetic solvent consisting of 160 g. of m-cresol, 160 g. of tetrahydronaphthalene, 20 g. of naphthalene, 10 g. of 1-methylnaphthalene, and 10 g. of gamma-picoline. The inorganic fraction of the solvent/solute system is 30 g. of water, 18 g. of NaOH, 4.5 g. of Na₂C0₃, and 30 g. Na₂S.9H₂0. The feed materials are reacted at 340°C, 1312 psia (8.99 MPa), 0.5 SLM of 95 percent carbon monoxide and 5 percent argon for 30 minutes. The results of the selective solvent extraction procedure are shown in Table 14.

### Example XIII

The foregoing procedure of Example XII is repeated, except that the organic fraction of the solvent/ solute system is 360 g. of synthetic solvent consisting of 260 g. of m-cresol, 60 g. of tetrahydronaphthalene, 20 g. of naphthalene, 10 g. of 1-methylnaphthalene, and 10 g. of gamma-picoline. The results of the selective solvent extraction procedure are shown in Table 14.

Examples XII and Xlll show that acceptable liquefaction yields can be obtained when the organic fraction of the solvent/solute system consists of a mixture of alkaline/alkaline-earth metal compounds. They also show the importance of phenolic compounds in the organic fraction of the solvent/solute system. In Examples XII, where m-cresol is 44.4 percent of the organic fraction, the yield is 66.27 percent. In Example XIII, m-cresol is increased to 72.2 percent of the organic fraction, the yield is increased to 73.82 percent.

The mineral contents of coals used in Examples VI through XIII are presented in Table 15.

## Claims

1. A method of converting carbonaceous materials to fuel products under conditions of temperature and pressure which do not produce significant thermal bond rupture in the carbonaceous materials characterized by: contacting the carbonaceous material with a solvent/solute system consisting of
(a) an organic phase comprising a solubilizing agent containing more than about 50% by weight of an aromatic phenol, polycyclic phenol, substituted phenol and mixtures and derivatives thereof; and
(b) an inorganic phase comprising an aqueous solution of a compound having a cation selected from alkali and alkaline-earth metals; said contacting being conducted at a temperature less than about 460°C. and a pressure of at least 2.06 MPa (about 300 psia).

2. A method according to claim 1, characterized by one or more of the following features:
(a) said organic phase solubilizing agent is selected from o-cresol, m-cresol, p-cresol, catechol, resorcinol, naphthol and mixtures and derivatives thereof;
(b) said organic phase further comprises one or more organic constituents selected from polycyclic aromatic hydrocarbons, partially-hydrogenated polycyclic aromatic hydrocarbons and fully hydrogenated polycyclic aromatic hydrocarbons having from 1 to 4 carbon rings, said organic constituent preferably being selected from naphthalene, anthracene, phenanthrene, acenaphthalene, 1-methylnaphthalene, 2-methylnaphthalene, tetrahydronaphthalene, gamma-picoline, isoquinoline, dihydronaphthalene, decahydronaphthalene, 9,10-dihydroanthracene, 9,10-dihydrophenanthrene and mixtures and derivatives thereof;
(c) said organic fraction is in whole or in part derived from liquefied carbonaceous material;
(d) said compound in the inorganic phase is selected from alkali hydroxides, alkali carbonates, alkali bicarbonates, alkali nitrates, alkali sulfates, alkali sulfites, alkali sulfides, alkali formates and other alkali salts, alkaline-earth hydroxides, alkaline-earth carbonates, alkaline-earth bicarbonates, alkaline-earth nitrates, alkaline-earth sulfates, alkaline-earth sulfites, alkaline-earth sulfides, alkaline-earth-formates and other alkaline-earth salts, and mixtures thereof;
(e) said compound in the inorganic phase is selected from sodium hydroxide, sodium carbonate, sodium bicarbonate, sodium sulfate, sodium sulfide, sodium nitrate, potassium hydroxide, potassium carbonate, potassium bicarboante; potassium formate, calcium carbonate and mixtures thereof.
(f) said compound in the inorganic phase is present in an amount from 1 part to 40 parts per 400 parts by weight of the solvent/solute system;
(g) the aqueous phase includes water present in an amount from 5 parts to 60 parts per 400 by weight of the solvent/solute system; and preferably includes water present in an amount of from 15 parts to 40 parts per 400 parts by weight of the solvent/solute system;
(h) said solubilizing agent has a boiling point from 50°C to 400°C and is present in an amount from 50 to 100 percent by weight of the organic fraction of the solvent/solute system, preferably 50 to 75 percent by weight of the organic fraction of the solvent/solute system;
(i) said contacting takes place at a temperature of from 100°C to 400°C, more preferably 140°C to 360°C, most preferably 260°C to 360°C, and at a pressure of from at least 2.06 to 17.2 MPa (about 300 psia to about 2500 psia) and for a time period sufficient to produce hydrocarbon liquids from said carbonaceous material; and
(j) said pressure is from 3.45 to 10.35 MPa (about 500 psia to about 1500 psia).

3. A method according to Claim 1, characterized in that said carbonaceous material is contacted with an excess of a solvent/solute system in the range of from about 1.5 to 1 to 5 to 1 solvent/solute to carbonaceous material.

## Patentansprüche

1. Verfahren zum Unwandeln kohlenstoffhaltiger Materialien in Brennstoffprodukte unter Temperatur-und Druckbedingungen, welche keine signifikante thermische Bindungsspaltung in den kohlestoffhaltigen Materialen erzeugen, gekennzeichnet durch: in Kontakbringen des kohlenstoffhaltigen Materiales mit einem Solvens/gelöstem Stoff-System, das besteht aus:
a) einer organischen Phase, die ein löslichmachendes Agens enthält, das mehr als ungefähr 50 Gewichtsprozent eines aromatischen Phenoles, eines polyzyklischen Phenoles, eines substituierten Phenoles und Mischungen und Derivaten daraus enthält, und
b) eine anorganische Phase, die eine wässrige Lösung einer Verbindung enthält, die ein Kation besitzt, das aus Alkali- und Erdalkalimetallen ausgewählt ist, wobei das in Kontakbringen bei einer Tempeatur von weniger als ungefähr 460 Grad C und einem Druck von wenigstens 2.06 MPa (ungefähr 300 psia) durchgeführt wird.

2. Verfahren nach Anspruch -1, gekennzeichnet durch ein oder mehrere der folgenden Merkmale:
a) das löslich machende Agens der organischen Phase wird aus O-Kresol, M-Kresol, P-Kresol, Katechol (Katechin), Resorzin, Naphthol und Mischungen und Derivaten daraus ausgewählt;
b) die organische Phase enthält weiterhin ein oder mehrere organische Bestandteile, die aus polyzyklischen aromatischen Kohlenwasserstoffen, teilhydrierten polyzyklischen aromatischen Kohlenwasserstoffen und vollhydrierten polyzyklischen aromatischen Kohlenwasserstoffen, die 1 bis 4 Kohlenstoffringe besitzen, ausgewählt werden, wobei die organischen Bestandteile vorzugsweise aus Naphtalin, Anthrazen, Phenanthren, Acenaphthalin, 1-Methylnaphthalin, 2-Methylnaphthalin, Tetrahydronaphthalin, Gamma-Picolin, Isoquinolin, Dihydronaphthalin, Decahydronaphthalin, 9,10-Dihydroanthrazen, 9,10-Dihydrophenanthren und Mischungen und Derivaten daraus, ausgewählt werden;
c) die organische Fraktion im Ganzen oder teilweise aus verflüssigtem kohlenstoffhaltigem Material abegleitet ist;
d) die Verbindung in der anorganischen Phase aus Alkalihydroxyden, Alkalikarbonaten, Alkalibikarbonaten, Alkalinitraten, Alkalisulfaten, Alkalisulfiten, Alkalisulfiden, Alkaliformiaten und anderen Alkalisalzen, Erdalkalihydroxyden, Erdalkalikarbonaten, Erdalkalibikarbonaten, Erdalkalinitraten, Erdalkalisulfaten, Erdalkalisulfiten, Erdalkalisulfiden, Erdalkaliformiaten und anderen Erdalkalisalzen und Mischungen daraus, ausgewählt werden;
e) die Verbindung in der anorganischen Phase aus Natriumhydroxyd, Natriumkarbonat, Natriumbikarbonat, Natriumsulfat, Natriumsulfid, Natriumnitrat, Kaliumhydroxyd, Kaliumkarbonat, Kaliumbikarbonat, Kaliumformiat, Kalziumkarbonat und Mischungen daraus, ausgewählt werden;
f) die Verbindungen der anorganischen Phase in einer Menge von einem Teil bis vierzig Teilen per 400 .Gewichsteilen des Solvens/gelöstem Stoff-Systemes gegenwärtig ist;
g) die wässrige Phase Wasser in einer Menge von 5 Teilen bis 60 Teilen per 400 Gewichsteilen des Solvens/gelöstem Stoff-Systemes enthält; und vorzugsweise Wasser in einer Menge von 15 bis 40 Teilen per 400 Gewichsteilen des Solvens/gelöstem Stoff-Systemes enthält;
h) das löslichmachende Agens einen Siedepunkt von 50 Grad C bis 400 Grad C bestizt und in einer Menge von 50 bis 100 Gewichtsprozent der organischen Fraktion des Solvens/gelöstem Stoff-Stystems vorhanden ist, vorzugsweise 50 bis 75 Gewichsprozent der organischen Fraktion des Solvens/gelöstem Stoff-System;
i) das in Kontakt bringen bei einer Temperatur von 100 Grad C bis 400 Grad C, mehr bevorzugt bei 140 bis 360 Grad C, am meisten bevorzugt bei 260 bis 360 Grad C und bei einem Druck von wenigstens 2.06 bis 17.2 MPa (ungefähr 300 psia bis ungefähr 2500 psia) und für eine genügende Zeitdauer zum Herstellen von Kohlenwasserstoffflüssigkeiten aus dem kohlenstoffhaltigen Material stattfindet; und
j) der Druck zwischen 3.15 bis 10.35 MPa (ungefähr 500 psia bis ungefähr 1500 psia) beträgt.
3. Verfahren nach Anspruch 1, dadurch gekennzeichnet, daß das kohlenstoffhaltige Material mit einem Überschuß eines Solvens/gelöstem Stoff-Systems im Bereich von ungefähr 1,5 zu 1 bis 5 zu 1 Solvens/ gelöstem Stoff zu kohlenstoffhaltigem Material in Kontakt gebracht wird.

## Revendications

1. Procédé poru convertir des substances carbonées en produits liquides sous certaines conditions de température et de pression, ce procédé n'entraînant pas une rupture signifactive des liaisons thermiques dans les substances carbonées, caractérisé en ce que l'on met en contact les substances carbonées avec un mélange solvant/soluté comportant:
a) une phase organique comprenant un agent solvant contenant plus de 50% en poids de phénol aromatique, de phénol polycyclique, de phénol substitué, et de mélanges ou de dérivés de ces produits, et
b) une phase inorganique comportant une solution alcaline d'un composé ayant un cation choisi parmi les métaux alcalins et alcalino-terreux, cette mise en contact étant effectuée à une température inférieure à 460°C et à une pression d'au moins 2,06 nla (environ 300 psia).

2. Procédé selon la revendication 1, caractérisé par une ou plusieurs des phases suivantes:
a) ledit agent solvant de la phase organique est sélectionné parmi les substances suivantes comprenant: le o-crésol, m-crésol, p-crésol, le catechol, le résorcinol, le naphtol et leurs mélanges et leurs dérivés,
b) ladite phase organique comprend en outre un ou plusieurs composants organiques choisis parmi les hydrocarbures aromatiques polycycliques, les hydrocarbures aromatiques polycycliques partiellement hydrogénés et les hydrocarbures aromatiques polycycliques totalement hydrogénés ayant un à quatre cycles de carbone, ces composants organiques étant de préférance choisis parmi le naphtalène, l'anthracène, le phénantrène, l'acénaphtalène, le 1-méthylnaphtalène, le 2-méthylnaphtalène, le tétrahydronaphtalène, le gammapicoline, l'isoquinoline, le dihydronaphtalène, le décahydronaphtalène, le 9,10-dihydroanthracène, le 9,10-dihydrophénantrène ainsi que leurs mélanges et leurs dérivés,
c) ladite fraction organique est partiellement ou entièrement dérivée de substances carbonées liquifées,
d) ledit composant de la phase inorganique est sélectionné parmi les hydrocydes alcalins, les carbonates alcalins, le bicarbonates alcalins, les nitrates alcalins, les sulfates alcalins, les sulfites alcalins, les sulfures alcalins, les formates alcalins et d'autres sels alcalins, les hydroxdes alcalino-terreux, les nitrates alcalino-terreux, les sulfates alcalino-terreux, les sulfites alcalino-terreux, les sulfures alcalino-terreux, les formates alcalino-terreux et autres sels alcalino-terreux ainsi que des mélanges de ces composés,
e) ledit composé de la phase inorganique est choisi parmi l'hydroxyde de sodium, le carbonate de sodium, le bicarbonate de sodium, le sulfate de sodium, le sulfure de sodium, le nitrate de sodium, l'hydroxyde de potassium, le carbonate de potassium, le bicarbonate de potassium le formate de potassium, le carbonate de calcium ainsi que parmi les mélanges de ces composés,
f) ledit composé de la phase inorganique est présent dans une proportion de 1 à 40 parties pour 400 parties en poids de composé solvant/soluté,
g) la phase acquese contient de l'eau dans une proportion comprise entre 5 et 60 parties en poids pour 400 parties du composé solvant/soluté, et contient de préférence de l'eau dans une proportion de 15 à 40 parties pour 400 parties en poids du composé solvant/soluté,
h) ledit agent solvant a un point d'ébullition compris entre 50 et 400°C et est présent dans une proportion allant de 50 à 100% en poids de la fraction organique du composé solvant/soluté, et de préférence dans une proportion comprise entre 50 et 75% en poids de la fraction organique du composé solvant/soluté,
i) ladite mise en contact s'effectue à une température comprise entre 100 et 400°C, avantageusement entre 140 et 360°C et de préférence entre 260 et 360°C et à une pression comprise au moins entre 300 psia et 2'500 psia, pendant un temps suffisamment long pour produire des hydrocarbures liquides à partir des substances carbonées, et
j) ladite'pression est comprise entre 500 psia et 1'500 psia.

3. Procédé selon la revendication 1, caractérisé en ce que les substances carbonées sont mises en contact avec un excédent du composé solvant soluté dans une proportion comprise entre 1,5 à 1 et 5 à 1 du composé solvant/soluté par rapport aux substances carbonées.
